

# UNITED STATES PATENT OFFICE.

KARL P. McELROY, OF WASHINGTON, DISTRICT OF COLUMBIA, AND CARLETON ELLIS, OF NEW YORK, N. Y., ASSIGNEES TO FIREPROOF PRODUCTS COMPANY, A CORPORATION OF NEW JERSEY.

## FIREPROOF FIBER AND METHOD OF MAKING SAME.

No. 914,300.

Specification of Letters Patent.

Patented March 2, 1909.

Application filed April 20, 1905. Serial No. 256,676.

To all whom it may concern:

Be it known that we, KARL P. McELROY and CARLETON ELLIS, citizens of the United States, residing, respectively, in Washington, District of Columbia, and New York, county and State of New York, have invented certain new and valuable Improvements in Fireproof Fibers and Methods of Making the Same, whereof the following is a specification.

This invention relates to fibers saturated or impregnated with soft or fluent, incombustible, materials insoluble in water, and, to the process of so saturating or impregnating them, all as more nearly set forth hereinafter, particular points of novelty being distinctly set forth in the appended claims.

No organic material can be made fireproof in the strictest sense of that term, since all organic materials will decompose and char when heated sufficiently high; but they can be made flameproof or flame resisting; *i. e.*, so that they will neither ignite on contact with a flame nor themselves emit flame when heated for a moderate length of time. This is the commercial sense of the word fireproof and the one employed hereinafter.

Many methods have been proposed for fireproofing fibers, animal and vegetable. Those depending on the deposition of insoluble mineral materials in the pores, as in the treatment of wood with successive solutions of soluble silicates and mineral salts, have proved of little avail for fireproofing, the mineral matter often really aiding combustion by holding open passageways for gases and air against natural sealing by tarry decomposition products, or fusible ash ingredients. Fibers so treated have further the defect of harshness, brittleness and inelasticity, the mineral matters preventing the free gliding of the fibers over one another which is necessary to preserve the original character of the fiber as regards elasticity and strength. Such fibers are often also detrimental to the edge of cutting tools. Other methods depending on the saturation with such soluble salts as give off flame-diluting and flame-stifling vapors, like alum and the ammonia salts, fireproof fairly well but where such salts are not deliquescent and therefore exist in the wood, etc., in the solid form, the fibers so treated suffer from the same mechanical defects as fibers containing

the insoluble mineral matters hereinbefore mentioned. Hard mineral matter such as crystals, in the pores of fibers is eminently undesirable from a mechanical point of view. Fireproofing with deliquescent salts, like zinc chlorid, accomplishes that end alone very well since these bodies hold enough water to shield the fiber from the effects of heat for some time. But these salts as well as all other soluble salts have proved very undesirable in practice since they will readily wash out in exposed situations like deck planking, or on such floors as are frequently scrubbed. Furthermore, they have the defect of readily taking up or giving off water, keeping in hygrometric balance with the state of the atmosphere, thereby making woodwork, for example, fireproofed by their aid, apt to check and warp. Paneling so fireproofed is also likely to keep rooms damp. As for the many proposed schemes for fireproofing fiber with ordinary organic materials like chromated glue, they merely add fuel to the flames.

Our invention consists in filling the pores of fibers with fluent, water insoluble, normally non-volatile materials of a stable and incombustible nature, which while making such fibers fireproof, do not render them either harsh or hygroscopic. The fluent character of the substance used, which may be oily, waxy or soft within the purview of our invention, permits the individual fibers to slide on each other; lubricates them in fact; and prevents any harshness or brittleness of the product. Instead of deteriorating the fiber, our substances really increase its strength and value, acting like the wax of waxed thread. Being insoluble in water, the substances are not affected by the hygrometric condition of the atmosphere; are not susceptible of being washed out; neither do they tend to wander from one portion of a tissue to another, leaving one spot destitute and accumulating in another, as is often the case with the zinc chlorid type of fireproofers. Woodwork fireproofed according to our invention does not check or warp; neither does it make apartments damp. Fiber impregnated with our insoluble substances is of course also waterproof. Preferably a fluent, incombustible substance is used which is also capable of evolving flame-stifling vapors when heated, thereby diluting the combus-

tible decomposition products of wood, etc., beyond the flaming point.

As suitable for the purposes of this invention is regarded any insoluble stable, non-volatile fluent substance, be it either waxy or liquid, which is also insoluble in water and uninflammable and is non-volatile at normal temperatures. As particularly adapted have been found the chlorin substitution products of organic radicals, and especially those of the aromatic radicals. Those of the paraffin radicals are less well suited, being less stable. Only the higher members of the paraffin series give halogenated derivatives of the desired consistency and these, when containing useful percentages of halogen, tend to break down readily into simpler compounds. Preferably the chlorin products are used because of their cheapness, although where price is not an object, the bromin and iodin products may also be used. As they contain a larger percentage of the uninflammable halogen than the corresponding chlorin compounds, they are even more desirable where not too costly. Halogen derivatives of naphthalene and anthracene, because of their cheapness, stability and general fluent nature are well suited to the purposes of this invention. Halogenated derivatives may of course contain two or more halogens in the same molecule, as with chlorobromnaphthalenes. Oily amins may also be used, as well as their compounds with inorganic acids, in so far as these are fluent and insoluble in their nature. Halogenated amins, as for instance, chloronaphthalamin, are particularly useful since they evolve ammoniacal vapors as well as halogenated vapors on being heated, both having a flame-stiffling property. Many organic bodies, as the drying and undrying fat oils, add halogen by direct combination, forming bodies which, when stable, are useful for our purpose. Wood oil, for instance, directly adds iodin, chlorin and bromin, forming soft bodies, which we have found incombustible, and which may be used alone or in admixture with other substances herein specified. Linseed oil behaves in a similar way. Asphalt, asphalt oils and dead oil may also be usefully chlorinated, etc.

There are very many halogenated naphthalene and anthracene products described, all being more or less suitable, being soft in consistency, uninflammable, and emitting flame-stiffling decomposition products when heated with fiber to the charring point of the latter. The uninflammability is of course comparative and increases directly with the percentage of halogen present, being greatest with the high halogenated bodies, as for instance perchloronaphthalene,  $C_{10}Cl_8$ . The hexachloronaphthalene, though not quite so incombustible as the higher homologues, is amply so for practical purposes. This body is a true wax in its physical characters and it

can be molded between the fingers; is insoluble in water; is stable at common temperatures and emits flame-stiffling vapors of chlorinated products when brought into contact with flame or with bodies at a red heat.

Any fiber or fibrous body may be treated with the described substances: wood, cloth, thread or rope, leather, paper, scenery, insulations, etc. By impregnating hide with these waxy and oily bodies, a true tawed leather which is also flame proof may be readily obtained.

In fireproofing with these halogenated bodies, they can be directly applied to wood in position, as in floors, paneling, furniture, etc., as any other oil or wax is applied; or they may be dissolved in any appropriate solvent, the fiber saturated with the solution, and the solvent distilled off. Using hexachloronaphthalene, it may be simply softened or liquefied by heat and worked into the pores of the wood, etc., with brushes and similar tools. As it cools, it forms a surface impregnation which prevents adjacent tissue from being reached by flame. By drying and heating the wood, etc. a complete saturation may of course be attained where such is deemed desirable. Bodies which have been melted or softened by heat and then again solidified are not porous, as in the case with all films deposited from solutions, and therefore when a surface is impregnated with hexachloronaphthalene, or a similar body, in the manner described, it closes all the pores of wood, etc., completely; seals it hermetically. Such being the case, where cheapness of treatment is an object, wood, etc., may first be saturated with water, or a watery fireproofer, such as a solution of zinc chlorid, ammonium phosphate, etc., and then sharply dried. This forms a dry surface layer and a wet interior, and said surface layer may then be impregnated with one of aforesaid fluent, insoluble fireproofers, particularly with the hexachloronaphthalene, thereby forming a hermetic surface sealing which completely encloses and protects such aqueous fireproofer from evaporation or hygrometric change.

In fireproofing cloth, ladies' dresses, etc., the fluent fireproofers of this invention may be usefully employed in lieu of paraffin in the ordinary sizing compositions, thereby rendering the cloth uninflammable without rendering it harsh.

In practice, in using the naphthalene derivatives, we preferably employ a mixture of the naphthalene chlorids, approaching as nearly as may be the hexachloro derivation, to save the tedious and unprofitable labor of separating the chemically pure bodies. By properly conducting the chlorination oily bodies can be obtained, but we prefer to form the waxy derivatives. Such mixtures of chlorinated bodies may be formed by exposing naphthalene hot to the action of chlorin gas,

either in the presence or absence of such chlorin carriers as antimony chlorid, chlorination being carried on till a body of the desired waxy consistence and flame resisting properties is obtained. Another and desirable method of obtaining these bodies is described and claimed in our co-pending application Ser. No. 295,730, filed Jan. 12, 1906, such method consisting essentially in chlorinating with electrolytic halogen. Preferably however, in using naphthalene bodies we carry on the chlorination nearly or quite to the point of forming the hexachlorid, such hexachlorid having desirable properties, as stated, and being more flame proof than lower halogenated bodies, sufficiently so to obviate any advantage in forming the hepta and octo chlorids, both bodies of less desirable mechanical properties. Additive chlorin derivatives of naphthalene may also be employed where the presence of more loosely bound chlorin is not detrimental.

What we claim and desire to secure by Letters Patent of the United States is:

- 25 1. Fiber impregnated and fireproofed with an incombustible, water-insoluble, stable, normally non-volatile, fluent substance, substantially as described.
- 30 2. Fiber impregnated and fireproofed with an incombustible, water-insoluble waxy substance, substantially as described.
- 35 3. Fiber superficially impregnated and fireproofed with an incombustible, normally non-volatile, stable, water-insoluble, fluent substance, substantially as described.
- 40 4. A mass of fiber superficially impregnated with an incombustible, water-insoluble material and interiorly impregnated with a watery fireproofer, substantially as described.
- 45 5. Fiber impregnated with stable, fluent, normally non-volatile halogen derivatives of organic bodies, substantially as described.
- 50 6. Fiber impregnated and fireproofed with a halogen derivative of naphthalene, substantially as described.
7. Fiber impregnated and fireproofed with chlorinated naphthalene, substantially as described.
- 50 8. Fiber impregnated and fireproofed with hexachlornaphthalene, substantially as described.

9. The process of treating fiber which consists in reducing a fluent, water-insoluble incombustible material to a liquid form and soaking said fiber therewith. 55

10. The process of fireproofing fiber which consists in impregnating a mass of fiber with a watery fireproofer, sharply drying the surface and then impregnating said surface with an incombustible, water-insoluble material, whereby said watery fireproofer is hermetically sealed within the interior, substantially as described. 60

11. The process of treating fiber which consists in reducing a fluent normally non-volatile, water-insoluble and stable halogen derivative of organic materials to a liquid form and soaking it into said fiber. 65

12. The process of treating fiber which consists in soaking into the surfaces of said fiber a halogen derivative of naphthalene in fluid form. 70

13. The process of treating fiber which consists in soaking into the surfaces of said fiber a chlornaphthalene in fluid form. 75

14. The process of treating fiber which consists in converting hexachlornaphthalene into a fluid form and soaking said fiber therewith. 80

15. The process of fireproofing fiber which consists in impregnating said fiber with an incombustible, water-insoluble, stable, fluent, normally non-volatile material. 85

16. The process of fireproofing fiber which consists in further softening a halogen derivative of naphthalene by heat and working it into the pores of said fiber while hot. 90

17. The process of fireproofing wood which consists in melting hexachlornaphthalene and working it into the pores of the wood. 95

18. The process of fireproofing fiber which consists in impregnating such fiber with an incombustible, water-insoluble, fluent, chlorination product of naphthalene containing hexachlornaphthalene. 95

In testimony whereof we affix our signatures, in presence of two subscribing witnesses.

KARL P. McELROY.  
CARLETON ELLIS.

Witnesses:

JNO. E. PARKER,  
J. H. JOCHUM, Jr.